# EUROPEAN PATENT SPECIFICATION

(11) **EP 2 528 704 B1**
(45) Date of publication and mention of the grant of the patent: **03.10.2018**
(21) Application number: 11736667.4
(22) Date of filing: 25.01.2011
(51) Int. Cl.: C25B 1/00, C25C 5/02, B22F 9/24

(54) **METHOD AND ARRANGEMENT FOR PRODUCING METAL POWDER**
VERFAHREN UND ANORDNUNG ZUR HERSTELLUNG EINES METALLPULVERS
PROCÉDÉ ET DISPOSITIF POUR PRODUIRE UNE POUDRE MÉTALLIQUE

(30) Priority: 29.01.2010 FI 20105083
(43) Date of publication of application: 05.12.2012
(73) Proprietor: OUTOTEC (FINLAND) OY, 02230 Espoo (FI)
(72) Inventor: NIEMINEN, Ville, FI-28300 Pori (FI); VIRTANEN, Henri, FI-28610 Pori (FI)
(74) Representative: Papula Oy
(86) International application number: PCT/FI2011/050056
(87) International publication number: WO 2011/092375

(56) References cited:
- EP-A1- 0 221 685
- EP-A1- 1 552 896
- FI-B- 120 438
- JP-A- 2002 327 289
- JP-A- 2003 328 198
- US-A- 4 789 444
- US-A- 5 882 502
- US-A1- 2005 067 299

## Description

### FIELD OF THE INVENTION

The invention relates to the production of finely divided metal powder. In particular, the invention relates to a dissolution-precipitation method and arrangement for producing metal powder.

### BACKGROUND OF INVENTION

Generally the end product in many metal manufacturing processes is a plate-like object in cathode form. This kind of end product is obtained for example by means of pyrometallurgical production routes utilizing electrolysis. In these methods, a metal anode that is pyrometallurgically made of a concentrate is electrolytically refined to cathode copper, which can for example be cast into products with various different forms. These types of methods can be used for producing copper, nickel or cobalt products, among others.

However, in the production of metals, in many cases it would be advantageous for instance with respect to further processing, if the metal received as the end product of the manufacturing process would be obtained in some other form than as a uniform solid object, such as a cathode plate. Particularly methods where the end product is obtained as pure metal powder would be extremely useful.

In the patent application JP2002327289, there is introduced a method for producing copper powder in electrolysis. In the method, an aqueous solution of sulfuric acid, containing titanium cathodes, is conducted to an anode chamber, so that the titanium cathodes reduce the copper dissolved in the anode chamber, thus precipitating it in the anode chamber into finely divided copper powder. The problem with this method is that the catholyte solution is conducted directly to the anode chamber, wherefore it is not possible to effectively control the mixture ratios of the catholyte solution and the anolyte solution. Moreover, in the method copper is precipitated directly into the anode chamber, which makes it more troublesome to remove the precipitated copper from the electrolytic arrangement. These problems constitute a risk for the creation of copper agglomerates, which makes it more difficult to control the particle size of copper powder.

The patent publication US2005/0023151 introduces a method where copper powder is made by electrolytically precipitating copper from copper sulfate on a cathode. The method makes use of a ferrous/ferric anode reaction, by which the energy consumption of the method is reduced. Said publication also describes a through-flow arrangement where the precipitated copper powder is recovered from the electrodes by means of an electrolyte flowing through the electrodes. A drawback with the method and arrangement illustrated in the publication US2005/0023151 is, among others, an unreliable recovery of copper from the cathodes, owing for example to the precipitation of copper in various different locations in the chamber containing electrodes, and to the attachment of copper on the cathode. Owing to the above mentioned drawbacks, among others, it is difficult to control the grain size of copper powder and of the morphology of copper particles, as well to achieve a homogeneous quality with separate electrodes. In addition, the precipitation of copper directly onto the cathode also depends on the cathode material and on the surface morphology, which in part increases the unreliability of the method.

The patent application WO2008/017731 introduces a method for manufacturing metal powder. In this method, valuable metal powder is precipitated by reducing the valuable metal dissolved in the method by means of another metal. In said method, also the dissolution of precious metal takes place in a reaction with said other metal, which weakens the control of the process kinetics as well as the efficiency thereof, and makes the method and the arrangement used therein fairly complicated.

Further, document US2005/067299 discloses an electrolytic method in diaphragm-type cell; document EP1552896 discloses a method for producing fine metal powder; document JP2003328198 discloses a method of generating copper ion and apparatus thereof; document EP0221685 discloses an electrolytic process for the manufacture of salts; and US5882502 discloses an electrochemical system and method.

### OBJECT OF INVENTION

The object of the invention is to eliminate above mentioned drawbacks of the prior art and to set forth a new method and arrangement for manufacturing metal powder in a solution-precipitation method making use of electrolysis.

### SUMMARY OF INVENTION

The method according to the invention is characterized by what is set forth in the independent claim 1.

The arrangement according to the invention is characterized by what is set forth in the independent claim 15.

In the method according to the invention for manufacturing metal powder, dissolved yield metal is mixed with a solution containing at least one intermediary metal for precipitating the dissolved yield metal into a yield metal powder. In the method, a first part of an acid-containing starting solution is brought to the anode side of the electrolytic cell as an anolyte, to be in contact with the anode and the supply material containing yield metal, and a second part of the acid-containing starting solution, which also contains intermediary metal in addition to acid, is brought to the cathode side of the electrolytic cell, as a catholyte to be in contact with the cathode; the yield metal is oxidized and dissolved in the anolyte by conducting electric current to the anode; the intermediary metal contained in the second part of the starting solution is reduced on the cathode side; and anolyte solution and catholyte solution are brought into a precipitation chamber for mixing the oxidized yield metal dissolved in the first part of the starting solution and the second part of the starting solution containing reduced intermediary metal.

The arrangement according to the invention is an arrangement for producing metal powder by precipitating yield metal powder by mixing dissolved yield metal powder with a solution containing at least one intermediary metal. The arrangement according to the invention comprises an electrolytic cell for dissolving the yield metal located on the anode side of the electrolytic cell and for oxidizing it in the anolyte, and for reducing, on the cathode side, the dissolved intermediary metal located on the cathode side of the electrolytic cell; a precipitation chamber arranged essentially separately from the electrolytic cell; as well as means for feeding anolyte solution and cathode solution respectively from the anode side and the cathode side of the electrolytic cell to the precipitation chamber for mixing the oxidized yield metal that is dissolved in the anolyte, and the cathode solution containing reduced intermediary metal, outside the electrolytic cell.

Among the advantages of the invention, let us point out for example good controllability of the particle size of the precipitating yield metal powder, which is made possible particularly by the feeding of the anolyte solution and cathode solution, to be mixed together, in a separate precipitation chamber, in which case the mixing ratio of said solutions can be controlled easily and accurately, as well as optimized according to the process conditions. Moreover, when the precipitation step takes place in a separate precipitation chamber, away from the vicinity of the electrodes, the effect of the electrodes in the precipitation process and in collecting the precipitate can be minimized, so that the reliability of the process is improved. Also the recovery of the yield metal precipitate becomes easier and more reliable. With a correct mixing ratio and an effective precipitate recovery, the creation of yield metal agglomerates can be prevented in the precipitation step, and consequently the homogeneity of the yield metal particles contained in the powder is enabled with respect to their size. A correct mixing ratio also facilitates a process with a better efficiency, which can be utilized for reducing the amount of energy needed in the process for producing a certain quantity of yield metal mass.

Unless otherwise stated, in the present document the expressions "anode side" and "cathode side" refer to those parts of the electrolytic cell that contain anolyte or catholyte in the vicinity of the anode or cathode, respectively. The "anode side" or the "cathode side" need not be a uniform part of the electrolytic cell, but the "anode side" or the "cathode side" may consist of several mutually separate elements comprising an anode or a cathode and anolyte or catholyte, respectively.

Unless otherwise stated, in the present document the expression "diaphragm" refers to any suitable film or thin mechanical obstacle, such as a membrane, an industrial textile or the like.

Unless otherwise stated, in the present document the expression "oxidation state", "oxidation level" or a corresponding expression refers to a charge level where an atom appears alone or apparently in a molecule. Thus the expressions "oxidation state", "oxidation level" or a corresponding expression can also refer to the apparent charge of an atom.

In an embodiment of the invention, the first part of the starting solution contains intermediary metal for boosting the dissolution of yield metal on the anode side. The first part of the circulating solution created as a result of mixing the anolyte solution and the catholyte solution is returned to anolyte. The first part of the starting solution is composed of the first part of the circulating solution. The second part of the circulating solution created as a result of mixing the anolyte solution and the catholyte solution is returned to catholyte. The second part of the starting solution is composed of the second part of the circulating solution. Moreover, in an embodiment of the invention, the circulating solution is returned essentially completely back to electrolyte, in which case the circulating solution is essentially composed of the first part of the circulating solution and of the second part of the circulating solution. When an anolyte solution that is formed of the first part of the starting solution and a catholyte solution that is formed of the second part of the starting solution are mixed together, there is created yield metal powder as the yield metal that was oxidized and dissolved in the anolyte is reduced, and the intermediary metal that was reduced in the catholyte is oxidized. The obtained circulating solution is recirculated in an arrangement to be used in the process in one of the embodiments of the invention, so that the circulating solution is partly or completely, after the mixing step and after the yield metal precipitate is separated from the solution, returned back to anolyte and/or catholyte. Now the intermediary metal is again reduced in the catholyte. Thus it is possible to realize an electrolytic regeneration of the intermediary metal in the catholyte, which means that in some embodiments of the invention, it is essentially not necessary to feed in the process new solution containing intermediary metal. In addition, when also the anolyte in some embodiments of the invention contains intermediary metal, said intermediary metal intensifies the dissolution of the yield metal in such process conditions, for example with relatively low acid contents, where dissolution with the combined effect of electric current and acid solution would not be efficient.

In an embodiment of the invention, the anolyte and the catholyte are mechanically separated by an electroconductive diaphragm. In an embodiment of the invention, the electrolytic cell comprises an electroconductive diaphragm provided in between the anode side and the cathode side of the electrolytic cell for mechanically separating the anode side and the cathode side.

Further, in an embodiment of the invention, an electroconductive separator solution is conducted in between the two diaphragms separating the anolyte and the catholyte in order to prevent a premature mixing of the anolyte and the catholyte. In an embodiment of the invention, the electrolytic cell comprises two electroconductive diaphragms provided in between the anode side and the cathode side of the electrolytic cell for mechanically separating the anode side and the cathode side by means of an electroconductive separator solution placed in the space between the two diaphragms.

In order to efficiently separate the precipitation step from the electrolytic cell and to realize this step in a controlled fashion and essentially completely in a separate precipitation chamber, the anolyte and the catholyte can in an embodiment of the invention be separated by means of an electroconductive diaphragm. In this document, the term "electroconductive diaphragm" refers to a diaphragm that is electroconductive to such extent that the diaphragm facilitates an effective operation of the electrolytic cell. However, in some embodiments of the invention, the electroconductivity of the diaphragm may be lower than the electroconductivity of those solutions that are mechanically separated by the diaphragm. Consequently, the purpose of the diaphragm is to mechanically separate the solutions located on different sides of the diaphragm, i.e. to serve as a mechanical obstacle, while at the same time being electroconductive to that extent that the electrolytic cell is capable of functioning effectively. This diaphragm divides the electrolytic cell to an anode part (or anode side), where the anolyte is located, and to a cathode part (or cathode side), where the catholyte is located. Thus the anolyte and the catholyte cannot be mixed together without disturbing the anode and cathode reactions, and metal powder cannot be formed in the vicinity of those electrodes in the electrolytic cell. For further intensifying the separation of the anode and the cathode, it is possible to use in between the anode side and the cathode side two partition diaphragms, and a separator solution can be fed in between said diaphragms.

In an embodiment of the invention, the yield metal is copper. In an embodiment of the invention, the yield metal is selected among the following group: nickel, cobalt, zinc, silver, gold, ruthenium, rhodium, palladium, osmium, iridium, platinum, manganese, zirconium, tin, cadmium and indium.

In an embodiment of the invention, the intermediary metal is vanadium. Further, in an embodiment of the invention, the intermediary metal is selected among the following group: titanium, chromium and iron. Further, in an embodiment of the invention, the intermediary metal is selected among the following group: manganese, zirconium, molybdenum, technetium, tungsten, quicksilver, germanium, arsenic, selenium, tin, antimony, tellurium and copper. In the various embodiments of the invention, the yield metals and intermediary metals can be selected among a group that depends on various different process parameters, particularly on the pH value of the electrolyte (i.e. on the oxygen content). On the basis of this description of the invention, a man skilled in the art is capable of finding in the above enlisted groups a suitable intermediary metal for a certain yield metal by means of routine testing. In particular, it has been found out that for example copper powder can be efficiently and reliably produced in an embodiment of the invention, when the selected intermediary metal is vanadium.

In an embodiment of the invention, the supply material containing yield metal is placed in the anode. Further, in an embodiment of the invention, the yield metal located on the anode side of the electrolytic cell is placed in the anode of the electrolytic cell. When the supply material containing yield metal is placed in the anode, the rate per unit of time of the electric current passing through the yield metal, and consequently also the mass of the dissolving yield metal per unit of time, can be efficiently controlled. The advantage of this embodiment is a particularly precise control of the dissolving reaction by means of electricity; yield metal is dissolved accurately according to the used quantity of electricity in the course of the given time period according to Faraday's laws. Moreover, the kinetics in the dissolution step are rapid, as the quantity of yield metal dissolved in the anolyte is directly proportional to the charge that has flown through the anode. Thus also the quantity of yield metal that is dissolved in the anolyte can be efficiently and accurately controlled, which facilitates a more precise control of the process dynamics, and an improvement in reliability.

In an embodiment of the invention, the yield metal is selected so that the selected yield metal is dissolved in the anolyte as a soluble salt of the acid that is contained in the first part of the starting solution.

In an embodiment of the invention, the electrolytes are placed in an oxygen-free environment, in order to prevent the oxidation of the yield metal and/or intermediary metal that is contained in the electrolytes. This makes it easier to control the acid content of the electrolytes, which means that the balance of chemical reactions taking place in the different solutions of the process and containing for example yield metal and/or intermediary metal can be adjusted more accurately, which in turn improves the reliability and efficiency of the process, among others.

In an embodiment of the invention, the starting solution contains sulfuric acid. Further, in an embodiment of the invention the sulfuric acid content in the starting solution is at least 50 g/l and preferably within the range 50 g/l - 1,500 g/l. In an embodiment of the invention, the starting solution contains hydrochloric acid or nitric acid. Further, in an embodiment of the invention the hydrochloric acid content in the starting solution is within the range 15 g/l - 500 g/l. Yet in an embodiment of the invention the starting solution contains, in addition to hydrochloric acid, also alkaline chloride, the content of which in the starting solution is within the range 15 g/l - 500 g/l. The suitability of an acid in the starting solution depends, among others, on the supply material, the yield metal and the intermediary metal in question. In some embodiments of the invention, the solutions may also contain more than one acid. On the basis of this description of the invention, a man skilled in the art is capable, by routine testing, of finding a suitable acid for a certain supply material, yield metal and intermediary metal, and a suitable content for said acid. In particular, it has been found out that in some embodiments of the invention, a sulfuric acid content of the starting solution that is at least 50 g/l provides for an efficient oxidation of a copper anode and its dissolution in the anode, when the intermediary metal is vanadium. A suitable acid, and content for said acid, must be chosen so that the yield metal is dissolved from the supply material to the anolyte, instead of the oxidation of the intermediary metal. Therefore the anolyte pH (i.e. oxygen content) must be suitable. When the employed yield metal is copper, and the intermediary metal is vanadium, the oxygen content must be as high as possible.

In an embodiment of the invention, the electrolytic cell comprises at least one bag defined by a diaphragm in order to restrict the anolyte and/or catholyte inside the bag. Further, in an embodiment of the invention the electrolytic cell comprises means for conducting the separator solution from a space left in between two diaphragms to the anode side and/or the cathode side.

The above described embodiments of the invention can be freely combined with each other. Several different embodiments can be combined in order to create a new embodiment. A method or arrangement that the invention relates to can include one or several of the above described embodiments of the invention.

### DETAILED DESCRIPTION OF INVENTION

In the specification below, the invention is described with reference to the appended drawings, where
Figure 1 is a flowchart illustrating an embodiment of a method according to the invention,
Figure 2 is a schematical illustration of an embodiment of an arrangement according to the invention,
Figure 3 is a schematical block diagram illustrating an embodiment of a method according to the invention,
Figure 4 is a schematical illustration of an embodiment of the electrolytic cell in an arrangement according to the invention,
Figure 5 shows scanning electron microscope images (SEM images) of copper powder produced by an embodiment of the invention.

For the sake of simplicity, reference numbers referring to various elements of the invention remain the same in connection with corresponding repeated elements.

In the preparation step S1 of an embodiment of the method according to Figure 1, there is produced and fed into the electrolytic cell, both to the anode side and to the cathode side, acid-bearing starting solution, electrolyte solution, which contains intermediary metal in its high potential value (i.e. in a higher oxidation state). In the method it is essential that at least the second part of the starting solution, which is fed to the cathode side, contains said intermediary metal in its high potential value, because in step S2, in the catholyte there is carried out the reduction of the intermediary metal to its low potential value (i.e. to a lower oxidation state), i.e. the regeneration of the intermediary metal. Also the first part of the starting solution, i.e. the part that is fed as the anolyte, may contain intermediary metal in its high potential value. In some embodiments of the invention, the starting solution may contain two or even several different intermediary metals. In some embodiments of the invention, the first and second part of the starting solution are identical in composition. By this procedure, the possibility that the composition of the electrolytes would be changed after starting the process is minimized, which means that the operating point of the process is stabilized more rapidly, and the controllability of the process is improved.

The type of intermediary metal suited in the method essentially depends on the selected yield metal, which should be dissolved in the anolyte in step S2, and which is later precipitated into powder in the mixing step S3. The intermediary metal and the selected yield metal together define the other features of the starting solution suited in the method, particularly the acid contained in the solution, and content of said acid in the solution. For example, the pH value of the solution must be such that in the prevailing process conditions, on the anode side there is more advantageously carried out the oxidation of yield metal and its dissolution in the anolyte than the oxidation of the intermediary metal in the anolyte. This kind of process conditions, i.e. functional windows, can be found for many different pairs of yield metal and intermediary metal. In the light of the description of the present invention as well as in the light of the Pourbaix diagrams of various different intermediary metals and yield metals, the finding of these functional windows represents routine testing for a man skilled in the art.

The starting solution can be produced in many different ways, which depend, among others, on the suitable intermediary metal. One way is for example to dissolve, in an aqueous solution of a suitable acid, oxide containing the desired intermediary metal. When necessary, the acid content of the starting solution and the oxidation number of the dissolved intermediary metal can thereafter be adjusted to be suitable with respect to the starting solution. The adjusting of the oxidation number of the intermediary metal can be carried out for example electrolytically.

When the starting solution is formed in step S1, it is fed as electrolyte in an electrolytic cell, where supply material containing yield metal is located on the anode side. In a method according to Figure 1, after step 1, in step 2 yield metal is dissolved on the anode side of the electrolytic cell from the supply material to the anolyte, as the yield metal is at the same time oxidized, and on the cathode side the intermediary metal of the starting solution is reduced from a high potential value to a low potential value. Because of productional considerations, among others, it is advantageous that the intermediary metal content and the content of the dissolved yield metal in the solutions is as high as possible. Thus a certain solution volume gives more precipitated yield metal powder in the mixing step S3 than in a situation where the contents of the intermediary metal and/or dissolved yield metal in the solutions are low.

The method according to Figure 1 can be realized by means of an arrangement illustrated schematically in Figure 2, where the employed supply material is present as an anode 2, which provides for rapid kinetics in the dissolution of yield metal, while the dissolution of the supply material is directly proportional to the charge flowing through the anode 2. Now the dissolution reactions can be controlled particularly accurately by using electricity; in a given period of time, the mass quantity of yield metal dissolved and oxidized on the anode is accurately proportional to the employed quantity of electricity, according to Faraday's laws. Respectively, an equimolar quantity of the intermediary metal is regenerated (reduced) on the cathode. The arrangement of Figure 2 also comprises a cathode 4, an anode side 6 of the electrolytic cell, a cathode side 8, anolyte filtering equipment 10, a precipitation chamber 12, separator equipment 16, and cleaning equipment 18 for the circulating solution. The anolyte 1 and the catholyte 3 are mechanically separated by means of an electroconductive separator solution 5 placed in the intermediate space 11 and by means of two electroconductive diaphragms 7 that define the intermediate space. The purpose is to ensure that the yield metal cations created on the anode side and the intermediary metal that is reduced to a low-potential value on the cathode side do not get into mutual contact in the electrolytic cell. Thus yield metal powder cannot be precipitated directly on the anode or cathode side of the electrolytic cell, which would, in case it happened, weaken the controllability of the process for example as regards the particle size of the yield metal powder as well as the process efficiency, and in addition, the recovery of the yield metal powder would become more difficult. In order to improve the separation of the anolyte 1 and the catholyte 3, the separator solution 5 provided in the intermediate space 11 can also be maintained at a higher hydrostatic pressure than the anolyte 1 and the catholyte 3.

After step S2, in step S3, anolyte solution is conducted from the anode side of the electrolytic cell and catholyte solution is conducted from the cathode side thereof, for example by means of suitable pipes or in some other way, to the precipitation chamber 12, in a suitable ratio away from the vicinity of the electrodes 2, 4. Because anolyte solution and catholyte solution are conducted to a separate precipitation chamber 12, the mixing ratio of the solutions can be controlled easily and accurately, and it can be optimized according to the process conditions. With a correct mixing ratio and an effective precipitate recovery, the creation of yield metal agglomerates can be prevented in the precipitation step, and consequently the homogeneity, with respect to their size, of the yield metal particles contained in the yield metal powder 14 is ensured. A correct mixing ratio also facilitates a process with a better efficiency, which results in reducing the amount of energy needed in the process for producing a certain quantity of yield metal mass.

In the precipitation chamber 12, there is mixed, or there can be continuously mixed the anolyte solution and the catholyte solution conducted in the chamber 12. Prior to conducting the anolyte solution into the precipitation chamber 12, it can in some embodiments of the invention be also purified of metallic impurities and/or other possible impurities disturbing the yield metal precipitation process in an anolyte filtering equipment 10 that is suited for this purpose. As a result of the mixing process, the oxidized yield metal of the anolyte solution is reduced and precipitated into solid yield metal powder 14, at the same time as the intermediary metal reduced in the catholyte solution is oxidized back to its high-potential value. From the obtained circulating solution, there is separated, in step S4, yield metal for example by centrifuging the circulating solution in separator equipment 16 suited for the purpose.

When the yield metal powder 14 is recovered, the created circulating solution is recirculated back to the electrolytic cell in step S5, part of it into anolyte 1 and part into catholyte 3. Before conducting the circulating solution back to the electrolytic cell, any dissolved yield metal that is possibly left in the circulating solution is removed therefrom, as well as yield metal particles, in cleaning equipment 18 suited for this purpose. The cleaning operation can be carried out for example electrolytically by reduction and filtering. A thorough removal of yield metal, both dissolved and precipitated, from the circulating solution prior to recirculating the circulating solution back to the electrolytic cell is useful for the reliability of the process, for improving process efficiency and the controllability of the particle size of the yield metal powder.

In the above described method, the composition of the circulating solution is essentially identical with the composition of the starting solution, because in precipitation, the intermediary metal is oxidized back into its starting solution value, and the yield metal dissolved in the anolyte 1 on the anode side is precipitated and separated from the solution. Thus the circulating solution created in the method can be reused as a starting solution. If also the recirculating of the circulating solution back to anolyte and catholyte is carried out with the same ratio that was applied when a corresponding electrolyte was fed from the anode side and the cathode side to the precipitation chamber in step S3, an essentially closed electrolyte circulation can be used in the process, without a need to separately add/remove solution to or from the anode side 6 of the electrolytic cell, or to or from the cathode side 8.

In practice, the method of Figure 1 is generally realized as a continuous electrolyte circulation, as a result of which in the precipitation chamber 12 there is continuously accumulated yield metal powder 14 to be separated from the circulating solution and to be recovered, until the recirculation of the electrolyte solution (circulating electrolyte) in the arrangement is stopped, or when the yield metal contained in the supply material (anode 2) is completely dissolved in the electrolytic cell. When there is no more need to produce yield metal powder 14, or when the yield metal of the supply material is finished on the anode side 6 of the electrolytic cell, the recovered yield metal powder 14 is treated in a finishing treatment in step S6, and the process is stopped. In some other preferred embodiments of the invention, the finishing treatment for the recovered yield metal powder 14 can be carried out simultaneously with the other steps of the process, in the course of the process of separating yield metal powder 14 and feeding it to the finishing treatment equipment (not illustrated).

In an example according to Figure 3, illustrated as a block diagram, the employed intermediary metal is vanadium, which in its high-potential value is V³⁺ in cations. The employed yield metal is copper, which is located in the supply material serving as the anode 2. The starting solution containing the vanadium intermediary metal in V³⁺ cations can be produced for instance by dissolving vanadium oxide V₂O₃ for instance to an aqueous solution of sulfuric acid. When the starting solution that contains V³⁺ cations in an aqueous solution, the sulfuric acid content of said solution being for example within the range 50 g/l - 1500 g/l, is formed, its first part is fed to the anode side 6 of the electrolytic cell as the anolyte 1, and the second part is fed to the cathode side 8 as the catholyte 3. When electric current flows through the electrolytic cell, the V³⁺ cations are reduced on the cathode side 8 to V²⁺ cations in the catholyte 3, and copper is dissolved from the anode 2 to the anolyte 1 as oxidized Cu²⁺ cations. Consequently, the anode reaction is Cu⁰ -> Cu²⁺ 2e⁻, and the cathode reaction is V³⁺ + e⁻ -> V²⁺.

In the dissolution of copper and its oxidation in the anolyte 1, the intermediary metal may in some embodiments of the invention participate in corresponding reactions, thus improving both dissolution and oxidation, in such process conditions, for example with fairly low acid contents, where dissolution and oxidation with the combined effect of a mere electric current and an acid solution would not be efficient. Now the precise mechanism how the intermediary metal participates in the dissolution and oxidation of the yield metal depends on the selected yield metal and intermediary metal. In the above described example, when the yield metal is copper and the intermediary metal is vanadium, vanadium may be oxidized on the anode side 6 into an intermediary oxidation state V⁵⁺, which is even higher than the V³⁺ state, whereafter the V⁵⁺ reacts with copper, thus oxidizing and dissolving copper. Now the "over-oxidized" vanadium V⁵⁺ is reduced back to its original high-potential value V³⁺. On the anode side 6, a corresponding "overoxidation" to an intermediate oxidation state is also possible with other intermediary metals than vanadium.

Thereafter anolyte solution and catholyte solution are conducted and mixed in a suitable ratio, for example in the ratio 1:3, in the precipitation chamber 12, where copper is precipitated through the reaction 2V²⁺ + Cu²⁺ -> 2V³⁺ + Cu⁰. On the basis of this precipitation reaction, anolyte and catholyte are in theory needed in the mixing ratio 1:2, in order to make all V²⁺ and Cu²⁺ cations present in the solutions participate in the precipitation of copper. An optimal mixing ratio depends on the reaction state of the anode reactions and on the current efficiency, as well as on the reaction state and current efficiency of the cathode reactions.

As regards the efficiency and reliability of the process, it is useful to ensure that any remarkable amounts of V²⁺ and/or Cu²⁺ cations are not left in the circulating solution. In some embodiments of the invention, it is for example advantageous to try and make sure that all Cu²⁺ cations are consumed in the precipitation reaction, in which case the real mixing ratio of anolyte and catholyte can be 1:N, where N > 2. However, the value of the parameter N also depends on how the circulating solution is cleaned before feeding it back to the electrolytic cell. On the basis of the description of the present invention, the finding of a suitable mixing ratio is obvious routine testing for a man skilled in the art.

When copper is precipitated into powder 14 and separated from the rest of the solution by means of the separator equipment 16, the remaining circulating solution is cleaned in the cleaning equipment 18 of any copper that is possibly left in the solution in the separation process, both of solid copper and dissolved, unprecipitated Cu²⁺ cations. The cleaning can be carried out for example electrolytically by precipitating and filtering. After said chemical and mechanical cleaning, the remaining circulating solution is essentially the same in composition as the starting solution, containing as a result from the precipitation reaction vanadium cations V³⁺ and sulfuric acid in aqueous solution. This circulating solution is again divided in a suitable ratio into anolyte 1 on the anode side 6 and into catholyte 3 on the cathode side 8. After the above described regeneration, the same circulation electrolyte can again be conducted through the arrangement and the method for precipitating more/new copper powder 14 to the precipitation chamber 12.

The solid yield metal powder 14 separated from the solution is finished (Figure 1, step S6) in a finish treatment arrangement. The separation and finish treatment processes can include many different steps, depending on the desired properties of the end product. In some embodiments of the invention, the yield metal powder 14 separated from the circulation electrolyte is washed in water for minimizing impurities carried along from the solution, whereafter the yield metal powder 14 is dried and coated with a passivation layer for preventing an oxidation of the powder, among others. In order to minimize the redissolution of the precipitated yield metal powder 14 back into the circulating solution, it is useful to perform the separation of the yield metal powder 14 from the circulating electrolyte by the separator equipment 16, and it is advisable to perform the washing as quickly as possible after the precipitation reaction.

In some embodiments of the invention, the yield metal powder 14 is subjected to various separate washing operations. In between the washing operations, the yield metal powder 14 is separated from the washing liquid. In an embodiment of the invention, the yield metal powder 14 that is obtained from the separator equipment 16, which is separated from the circulating electrolyte by centrifuging but is still wet, is mixed in water in the mass mixing ratio 1:20 (one part of wet yield metal powder 14 and 20 parts of water) three times. In between the mixing operations, the yield metal powder 14 is separated from the washing liquid.

The exact structure and operation of the washing equipment can vary even to a great extent, and for a man skilled in the art, the production of such equipment is obvious in the light of the description of the present invention. In a preferred embodiment of the invention, the washing equipment for realizing several successive washing operations can be for example a conveyor-belt type arrangement, where the wet yield metal powder 14 is poured on a conveyor belt, which conveys the yield metal powder 14 to the washing liquid, from which the yield metal powder is poured on the next conveyor belt, etc. Now the settling of the yield metal powder 14 takes place when it is separated from the washing liquid, i.e. when the washing liquid containing yield metal powder is poured on the conveyor belt.

In addition to the above described example, or instead of the procedure described therein, the separated yield metal powder can naturally also be washed by many known methods, for example by means of a syphon.

Various different electrolytic cell structures can be designed for dissolving and oxidizing yield metal on the anode side of an electrolytic cell, and for reducing intermediary metal on the cathode side of an electrolytic cell. The electrolytic cell structure illustrated schematically in Figure 4 can be used in the arrangement for producing yield metal powder 14 in a reliable and efficient way, with a good efficiency.

In the electrolytic cell of Figure 4, both the anode side 6 and the cathode side 8 comprise several sections, i.e. diaphragm bags, defined by a diaphragm 7. Each diaphragm bag respectively includes an anode 2 or a cathode and anolyte 1 or catholyte 3. Naturally the anodes 2 and the cathodes 4 are connected to a power source (not illustrated). In between each diaphragm bag, there is supplied electroconductive separator solution 5, which in one embodiment of the invention contains intermediary metal in a suitable high-potential value, i.e. in an oxidized state; in the case of the above described example, the separator solution 5 may contain for example V³⁺ ions.

In addition, the electrolytic cell of Figure 4 comprises a feed pipe 9 for feeding separator solution to the intermediate space 11 left between the diaphragm bags, an overflow channel 13 for the separator solution 4, drain channels 15 for the anolyte solution and the catholyte solution, as well as a protective film 17. The electrolytic cell of Figure 4 can be connected to another arrangement, for example to a precipitation chamber 12 (not illustrated in Figure 4), by intermediation of the drain channels 15 and the feed pipe 9.

In an embodiment of the invention, the separator solution 5 serves as the starting solution, in which case the composition of the separator solution 5 is identical to that of the starting solution. Now the starting solution can be fed to the intermediate space 11 of the electrolytic cell illustrated in Figure 4 through the apertures provided in the feed pipe 9. From the intermediate space 11, the separator solution 5 flows to the diaphragm bags as anolyte 1 and catholyte 3 through perforations provided in the diaphragms 7. In addition or instead, the diaphragm can be semi-permeable, so that the separator solution 5 (starting solution) has access to flow in a controlled fashion through the diaphragm 7 as anolyte 1 and/or catholyte 3. Anode reactions and cathode reactions take place in the diaphragm bags in the way described above. The obtained catholyte solution, containing reduced intermediary metal, as well as the anolyte solution containing dissolved or oxidized yield metal, can be conducted to the precipitation chamber 12 for example through outlets 15. In some embodiments of the invention, the outlets 15 can serve as overflow channels for removing excess electrolyte from the arrangement, in which case anolyte solution and/or catholyte solution can be brought in the precipitation chamber 12 via another route, for example through suction inlets provided for this purpose. The circulating solution created in the precipitation chamber 12 can in turn be recirculated, after possible cleaning steps, for example via a feed pipe 9 back to the intermediate space 11 and further to anolyte 1 and/or catholyte 3.

By adjusting the permeability of the diaphragms 7 in the cell illustrated in Figure 4, or the size of the perforations provided in the diaphragms 7, the quantity of the solution flowing through the anode side 6 and/or the cathode side 8 per unit of time can be efficiently controlled. The permeability of the diaphragms 7 can be selected separately for the diaphragms 7 on the anode side 6 and/or for the diaphragms 7 on the cathode side 8. By suitably controlling the quantity of solution per time unit that has access to flow in the diaphragm bags on the anode side 6 and/or on the cathode side 8 through the diaphragms 7, in relation to the quantity of solution per time unit to be fed in the intermediate space 11, the hydrostatic pressure of the separator solution 5 placed in the intermediate space 11 can be adjusted to be higher than the hydrostatic pressure of the electrolytes contained in the diaphragm bags located in the separator solution 5. Thus it is possible to prevent an undesired flowing of the electrolyte through the diaphragm 7 towards the intermediate space 11, away from the diaphragm bag. By suitably arranging the measures of the overflow channel 13, for example by arranging it at a suitable height, it is possible to ensure according to Figure 4 that the hydrostatic pressure difference between the intermediate space 11 and the anode side 6 and/or the cathode side 8 does not rise too high, but any excess separator solution flows out of the cell through the overflow channel 13. Respectively, also by arranging the measures and locations of the outlets 15, it is possible to affect the formation of said hydrostatic pressure difference. When the diameter of the perforations possibly provided in the diaphragms 7 is large, said hydrostatic pressure difference, together with the permeability of the diaphragms 7, essentially defines the quantity of solution that flows through the anode side 6 and the cathode side 8 per unit of time. On the basis of the description of the present invention, the above described design of the measures of the electrolytic cell, and the placing of the perforations, is obvious routine testing for a man skilled in the art.

As was described above, in some embodiments of the invention it is not necessary to directly feed starting solution and/or circulating solution to the anode side 6 and/or cathode side 8 of the electrolytic cell, for example to the diaphragm bags, but essentially all solution in the arrangement circulates through the intermediate space 11. In case the diaphragms 7 are selected to be such that they are completely impermeable to solution, circulating solution and/or starting solution can be fed to the anode side 6 and/or to the cathode side 8, for example to the diaphragm bags, directly and not through the intermediate space 11. In some other embodiments of the invention, instead of the diaphragms 7, there can be used for example ion-selective membranes that only permeate ions of a certain type.

In the electrolytic cell according to Figure 4, the electrolytic cell structure is covered by a protective film 17, by means of which the intermediate space 11 can be pressurized for example with nitrogen gas or with some other inert gas in order to prevent a possible oxidation caused by air or the surrounding environment. Also the diaphragm bags can be closed and pressurized with nitrogen in order to prevent oxidation.

The cell structure of Figure 4 enables a reliable separation of the anolyte and the catholyte in the electrolytic cell, which reduces premature oxidation and/or reduction reactions. Consequently, by using the electrolytic cell structure according to Figure 4, there is achieved a good efficiency in the method. In addition, the risk of a premature precipitation of the yield metal powder in the electrolytic cell is reduced, which improves the reliability of the method and makes the maintenance of the equipment easier.

### EXAMPLE

By applying a method according to the block diagram illustrated in Figure 3, there was manufactured, in an arrangement representing essentially the type illustrated in Figure 2, copper powder by employing as the starting solution an aqueous solution of sulfuric acid, said solution containing V³⁺ cations. In this starting solution, the measured sulfuric acid concentration was about 500 g/l, and the measured vanadium concentration was about 16 g/l. The employed supply material was Class A cathode copper plate, which also served as the anode of the electrolytic cell. The employed cathode was a lead plate, measures 275 mm x 130 mm. In test conditions, the solution temperatures were roughly 20 - 35° C.

The starting solution was fed to the electrolytic cell, where copper anode was oxidized and dissolved in the anolyte. The measured content of the dissolved copper was roughly 4 g/l. Thereafter anolyte solution was conducted from the anode side, and catholyte solution was conducted from the cathode side to the precipitation chamber, which in this example was a glass bottle. The mixing ratio of the anolyte solution and the catholyte solution was 1:3. As a result of the mixing operation, copper powder was formed in the precipitation chamber, according to the description above. The electron microscope images taken of the obtained copper powder are illustrated in Figure 5; from these images it can be observed, for example, that the size distribution of the copper particles is fairly homogeneous, large particle agglomerates are not created, and the average size of the particles is below the micrometer range.

Although some examples and embodiments illustrating the invention are above described as methods for manufacturing copper powder, a man skilled in the art is on the basis of this description of the invention easily capable of manufacturing powders also of other metals than copper when applying the various embodiments of the invention. Likewise, on the basis of this description of the invention, a man skilled in the art is easily capable of using, in the various embodiments of the invention, other intermediary metals and/or acids than those enlisted in the above examples. The invention is not restricted to the above described examples only, but it can be realized in many different modifications within the scope of the appended claims.

## Claims

1. A method for manufacturing a yield metal powder, wherein dissolved yield metal is mixed with a solution containing at least one intermediary metal for precipitating the dissolved yield metal into the yield metal powder (14), wherein in the method
- a first part of an acid-containing starting solution is brought as an anolyte (1) to the anode side (6) of an electrolytic cell, to be in contact with the anode (2) and a supply material containing the yield metal; and a second part of the acid-containing starting solution, which also contains the intermediary metal, in a higher oxidation state, in addition to acid, is brought to the cathode side (8) of the electrolytic cell, as a catholyte (3) to be in contact with the cathode (4);
- the yield metal is oxidized and dissolved in the anolyte (1) by conducting electric current in the anode (2);
- the intermediary metal contained in the second part of the starting solution is reduced to a lower oxidation state on the cathode side (8);
- anolyte solution and catholyte solution are brought into a precipitation chamber (12) for mixing the oxidized yield metal dissolved in the first part of the starting solution and the second part of the starting solution containing the reduced intermediary metal;
- a first part of the circulating solution created as a result of mixing the anolyte solution and the catholyte solution is returned back to anolyte (1); wherein the first part of the starting solution is composed of the first part of the circulating solution; and
- a second part of the circulating solution created as a result of mixing the anolyte solution and the catholyte solution is returned back to catholyte (3); wherein the second part of the starting solution is composed of the second part of the circulating solution.

2. A method according to claim 1, **characterized in that** the first part of the starting solution contains the intermediary metal for boosting the dissolution of yield metal on the anode side.

3. A method according to claim 1 , **characterized in that** the circulating solution is conducted completely back to electrolyte, so that the circulating solution is composed of the first part of the circulating solution and of the second part of the circulating solution.

4. A method according to any of the claims 1-3, **characterized in that** the anolyte (1) and the catholyte (3) are mechanically separated by an electroconductive diaphragm (7).

5. A method according to any of the claims 1-4, **characterized in that** an electroconductive separator solution (5) is conducted in between two diaphragms (7) separating the anolyte (1) and the catholyte (3) in order to prevent a premature mixing of the anolyte (1) and the catholyte (3).

6. A method according to any of the claims 1-5, **characterized in that** the yield metal is copper.

7. A method according to any of the claims 1-5, **characterized in that** the yield metal is selected among the following group: nickel, cobalt, zinc, silver, gold, ruthenium, rhodium, palladium, osmium, iridium, platinum, manganese, zirconium, tin, cadmium and indium.

8. A method according to any of the claims 1-5, **characterized in that** the intermediary metal is vanadium.

9. A method according to any of the claims 1-5, **characterized in that** the intermediary metal is selected among the group titanium, chromium and iron.

10. A method according to any of the claims 1-5, **characterized in that** the intermediary metal is selected among the following group: manganese, zirconium, molybdenum, technetium, tungsten, quicksilver, germanium, arsenic, selenium, tin, antimony, tellurium and copper.

11. A method according to any of the claims 1-10, **characterized in that** the supply material containing the yield metal is located in the anode (2) .

12. A method according to any of the claims 1-11, **characterized in that** the starting solution contains sulfuric acid.

13. A method according to claim 12, **characterized in that** the content of sulfuric acid in the starting solution is at least 50 g/l and preferably 50 g/l - 1500 g/l.

14. A method according to any of the claims 1-13, **characterized in that** the starting solution contains hydrochloric acid or nitric acid.

15. An arrangement for producing a yield metal powder by precipitating the yield metal powder (14) by mixing dissolved yield metal with a solution containing at least one intermediary metal in a lower oxidation state, wherein the arrangement comprises an electrolytic cell containing yield metal on an anode side and dissolved intermediary metal on a cathode side, for dissolving the yield metal located on the anode side of the electrolytic cell and for oxidizing it in the anolyte, and for reducing the dissolved intermediary metal located on the cathode side (8) of the electrolytic cell on the cathode side from a higher oxidation state to the lower oxidation state; a precipitating chamber (12) that is separate from the electrolytic cell; as well as means for feeding anolyte solution and catholyte solution respectively from the anode side (6) of the electrolytic cell and from the cathode side (8) of the electrolytic cell to the precipitating chamber (12) for mixing the yield metal dissolved in the anolyte and the catholyte solution containing the reduced intermediary metal, from outside the electrolytic cell; and means for returning a first part of the circulating solution created as a result of mixing the anolyte solution and the catholyte solution back to anolyte (1); wherein the first part of the starting solution is composed of the first part of the circulating solution; and means for returning a second part of the circulating solution created as a result of mixing the anolyte solution and the catholyte solution back to catholyte (3); wherein the second part of the starting solution is composed of the second part of the circulating solution.

16. An arrangement according to claim 15, **characterized in that** the electrolytic cell comprises an electroconductive diaphragm (7) in between the anode side (6) and the cathode side (8) of the electrolytic cell for mechanically separating the anode side (6) and the cathode side (8).

17. An arrangement according to any of the claims 15-16, **characterized in that** the electrolytic cell comprises two electroconductive diaphragms (7) in between the anode side (6) and cathode side (8) of the electrolytic cell for mechanically separating the anode side (6) and the cathode side (8) by means of an electroconductive separator solution (5) provided in the space left between the two diaphragms (7).

18. An arrangement according to any of the claims 15-17, **characterized in that** the yield metal supplied on the anode side (6) of the electrolytic cell is located in the anode (2) of the electrolytic cell.

19. An arrangement according to any of the claims 15-18, **characterized in that** the electrolytic cell comprises at least one bag, defined by a diaphragm (7), for keeping the anolyte and/or the catholyte inside the bag.

20. An arrangement according to claim 17, **characterized in that** the electrolytic cell comprises means for conducting a separator solution (5) from the space left between the two diaphragms (7) to the anode side (6) and/or to the cathode side (8).

21. An arrangement according to any of the claims 15-20, **characterized in that** the electrolytes are placed in an oxygen-free environment for preventing the oxidation of the yield metal and/or intermediary metal contained in the electrolytes.

## Patentansprüche

1. Ein Verfahren zur Herstellung eines Streckmetallpulvers, bei dem gelöstes Streckmetall mit einer Lösung gemischt wird, die mindestens ein Zwischenmetall für das Abscheiden des gelösten Streckmetalls zu dem Streckmetallpulver (14) enthält,
wobei in dem Verfahren
- ein erster Teil einer säurehaltigen Ausgangslösung als Anolyt (1) auf die Anodenseite (6) einer Elektrolysezelle gebracht wird, um mit der Anode (2) und einem mit Streckmetall enthaltenden Versorgungsmaterial in Kontakt zu sein; und ein zweiter Teil der säurehaltigen Ausgangslösung, die auch das Zwischenmetall enthält, mit einer höheren Oxidationsstufe als Katholyt (3), neben der Säure, auf die Kathodenseite (8) der Elektrolysezelle gebracht wird, um mit der Kathode (4) in Kontakt zu sein;
- das Streckmetall oxidiert und im Anolyten (1) durch Leiten von elektrischem Strom in der Anode (2) gelöst wird;
- das Zwischenmetall, enthalten im zweiten Teil der Ausgangslösung, auf eine niedrigere Oxidationsstufe auf der Kathodenseite (8) reduziert wird;
- Anolytenlösung und Katholytenlösung in eine Fällungskammer (12) gebracht werden, um das im ersten Teil der Ausgangslösung gelöste oxidierte Streckmetall und den zweiten Teil der mit reduziertem Zwischenmetall enthaltener Ausgangslösung zu vermischen;
- ein erster Teil der zirkulierenden Lösung, die durch Mischen der Anolytenlösung und der Katholytenlösung entsteht, zum Anolyten (1) zurückgeführt wird; wobei der erste Teil der Ausgangslösung aus dem ersten Teil der zirkulierenden Lösung besteht; und
- ein zweiter Teil der zirkulierenden Lösung, die durch Mischen der Anolytenlösung und der Katholytenlösung entsteht, zum Katholyten (3) zurückgeführt wird; wobei der zweite Teil der Ausgangslösung aus dem zweiten Teil der zirkulierenden Lösung besteht.

2. Ein Verfahren nach Anspruch 1, **dadurch gekennzeichnet, dass** der erste Teil der Ausgangslösung das Zwischenmetall zur Verstärkung der Auflösung von Streckmetall auf der Anodenseite enthält.

3. Ein Verfahren nach Anspruch 1, **dadurch gekennzeichnet, dass** die zirkulierende Lösung vollständig zu den Elektrolyten zurückgeführt wird, so dass die zirkulierende Lösung aus dem ersten Teil der zirkulierenden Lösung und dem zweiten Teil der zirkulierenden Lösung besteht.

4. Ein Verfahren nach einem der Ansprüche 1-3, **dadurch gekennzeichnet, dass** der Anolyt (1) und der Katholyt (3) mechanisch durch eine elektrisch leitfähige Membran (7) getrennt sind.

5. Ein Verfahren nach einem der Ansprüche 1-4, **dadurch gekennzeichnet, dass** eine elektrisch leitfähige Trennlösung (5) zwischen zwei Membranen (7) zwischen dem Anolyten (1) und dem Katholyten (3) durchgeleitet wird, um eine vorzeitige Vermischung des Anolyten (1) und des Katholyten (3) zu verhindern.

6. Ein Verfahren nach einem der Ansprüche 1-5, **dadurch gekennzeichnet, dass** das Streckmetall Kupfer ist.

7. Ein Verfahren nach einem der Ansprüche 1-5, **dadurch gekennzeichnet, dass** das Streckmetall aus der folgenden Gruppe: Nickel, Kobalt, Zink, Silber, Gold, Ruthenium, Rhodium, Palladium, Osmium, Iridium, Platin, Mangan, Zirkonium, Zinn, Cadmium und Indium ausgewählt wird.

8. Ein Verfahren nach einem der Ansprüche 1-5, **dadurch gekennzeichnet, dass** das Zwischenmetall Vanadium ist.

9. Ein Verfahren nach einem der Ansprüche 1-5, **dadurch gekennzeichnet, dass** das Zwischenmetall aus der Gruppe Titan, Chrom und Eisen ausgewählt wird.

10. Ein Verfahren nach einem der Ansprüche 1-5, **dadurch gekennzeichnet, dass** das Zwischenmetall aus der folgenden Gruppe: Mangan, Zirkonium, Molybdän, Technetium, Wolfram, Quecksilber, Germanium, Arsen, Selen, Zinn, Antimon, Tellur und Kupfer ausgewählt wird.

11. Ein Verfahren nach einem der Ansprüche 1-10, **dadurch gekennzeichnet, dass** sich das Versorgungsmaterial, das das Streckmetall enthält, in der Anode (2) befindet.

12. Ein Verfahren nach einem der Ansprüche 1-11, **dadurch gekennzeichnet, dass** die Ausgangslösung Schwefelsäure enthält.

13. Ein Verfahren nach Anspruch 12, **dadurch gekennzeichnet, dass** der Gehalt an Schwefelsäure in der Ausgangslösung mindestens 50 g/l und vorzugsweise 50 g/l - 1500 g/l beträgt.

14. Ein Verfahren nach einem der Ansprüche 1-13, **dadurch gekennzeichnet, dass** die Ausgangslösung Salzsäure oder Salpetersäure enthält.

15. Eine Vorrichtung zur Herstellung eines Streckmetallpulvers durch Fällung des Streckmetallpulvers (14) durch Mischen von gelöstem Streckmetall mit einer Lösung, die mindestens ein Zwischenmetall mit einer niedrigeren Oxidationsstufe enthält, wobei die Vorrichtung eine Elektrolysezelle mit Streckmetall auf einer Anodenseite und gelöstes Zwischenmetall auf einer Kathodenseite beinhaltet, zum Auflösen des Streckmetalls, welches sich auf der Anodenseite der Elektrolysezelle befindet, und um es im Anolyten zu oxidieren und um das gelöste Zwischenmetall an der Kathodenseite (8) der Elektrolysezelle an der Kathodenseite von einer höheren Oxidationsstufe zur niedrigeren Oxidationsstufe zu reduzieren; eine Fällungsskammer (12), die getrennt von der Elektrolysezelle ist; sowie Mittel für die Zuführung der Anolytenlösung und Katholytenlösung jeweils von der Anodenseite (6) der Elektrolysezelle und von der Kathodenseite (8) der Elektrolysezelle zur Fällungskammer (12) zum Mischen des Streckmetalls gelöst im Anolyten und die Katholytenlösung, die das reduzierte Zwischenmetall enthält, von außerhalb der Elektrolysezelle; und Mittel zur Rückführung eines ersten Teils der zirkulierenden Lösung, die durch das Mischen der Anolytenlösung und der Katholytenlösung zurück zum Anolyten (1) entsteht; wobei der erste Teil der Ausgangslösung aus dem ersten Teil der zirkulierenden Lösung besteht; und Mittel zur Rückführung eines zweiten Teils der zirkulierenden Lösung, die durch das Mischen der Anolytenlösung und der Katholytenlösung zurück zum Katholyten (3) entsteht; wobei der zweite Teil der Ausgangslösung aus dem zweiten Teil der zirkulierenden Lösung besteht.

16. Eine Vorrichtung nach Anspruch 15, **dadurch gekennzeichnet, dass** die Elektrolysezelle eine elektrisch leitfähige Membran (7) zwischen der Anodenseite (6) und der Kathodenseite (8) der Elektrolysezelle zur mechanischen Trennung der Anodenseite (6) und der Kathodenseite (8) umfasst.

17. Eine Vorrichtung nach einem der Ansprüche 15-16, **dadurch gekennzeichnet, dass** die Elektrolysezelle zwei elektrisch leitfähigen Membranen (7) zwischen der Anodenseite (6) und der Kathodenseite (8) der Elektrolysezelle zur mechanischen Trennung der Anodenseite (6) und der Kathodenseite (8) mittels einer elektrisch leitfähigen Trennlösung (5) umfasst, vorhanden in dem verbleibenden Raum zwischen den beiden Membranen (7).

18. Eine Vorrichtung nach einem der Ansprüche 15-17, **dadurch gekennzeichnet, dass** sich das an der Anodenseite (6) der Elektrolysezelle zugeführte Streckmetall in der Anode (2) der Elektrolysezelle befindet.

19. Eine Vorrichtung nach einem der Ansprüche 15-18, **dadurch gekennzeichnet, dass** die Elektrolysezelle mindestens einen Beutel, definiert durch eine Membran (7), zum Halten des Anolyten und/oder des Katholyten in dem Beutel umfasst.

20. Eine Vorrichtung nach Anspruch 17, **dadurch gekennzeichnet, dass** die Elektrolysezelle Mittel zum Leiten einer Trennlösung (5) von dem verbleibenden Raum zwischen den beiden Membranen (7) zur Anodenseite (6) und/oder zur Kathodenseite (8) umfasst.

21. Eine Vorrichtung nach einem der Ansprüche 15-20, **dadurch gekennzeichnet, dass** die Elektrolyte in einer sauerstofffreien Umgebung angeordnet sind, um die Oxidation des Streckmetalls und/oder Zwischenmetalls, enthalten in den Elektrolyten, zu verhindern.

## Revendications

1. Procédé pour fabriquer une poudre de métal de rapport, dans lequel le métal de rapport dissous est mélangé avec une solution contenant au moins un métal intermédiaire pour précipiter le métal de rapport dissous dans la poudre de métal de rapport (14),
dans lequel dans le procédé
- une première partie d'une solution de départ contenant un acide est apportée en tant qu'anolyte (1) jusqu'au côté anode (6) d'une cellule électrolytique, pour être en contact avec l'anode (2) et une matière d'alimentation contenant le métal de rapport ; et une seconde partie de la solution de départ contenant un acide, qui contient également le métal intermédiaire, dans un état d'oxydation supérieur, en plus de l'acide, est apportée jusqu'au côté cathode (8) de la cellule électrolytique, en tant que catholyte (3) pour être en contact avec la cathode (4) ;
- le métal de rapport est oxydé et dissous dans l'anolyte (1) en conduisant du courant électrique dans l'anode (2) ;
- le métal intermédiaire contenu dans la seconde partie de la solution de départ est réduit jusqu'à un état d'oxydation inférieur sur le côté cathode (8) ;
- une solution d'anolyte et une solution de catholyte sont apportées dans une chambre de précipitation (12) pour mélanger le métal de rapport oxydé dissous dans la première partie de la solution de départ et la seconde partie de la solution de départ contenant le métal intermédiaire réduit ;
- une première partie de la solution en circulation créée suite au mélange de la solution d'anolyte et de la solution de catholyte est renvoyée à l'anolyte (1) ; dans laquelle la première partie de la solution de départ est composée de la première partie de la solution en circulation ; et
- une seconde partie de la solution en circulation créée suite au mélange de la solution d'anolyte et de la solution de catholyte est renvoyée au catholyte (3) ; dans laquelle la seconde partie de la solution de départ est composée de la seconde partie de la solution en circulation.

2. Procédé selon la revendication 1, **caractérisé en ce que** la première partie de la solution de départ contient le métal intermédiaire pour augmenter la dissolution de métal de rapport du côté anode.

3. Procédé selon la revendication 1, **caractérisé en ce que** la solution en circulation est menée complètement en retour jusqu'à l'électrolyte, de sorte que la solution en circulation est composée de la première partie de la solution en circulation et de la seconde partie de la solution en circulation.

4. Procédé selon l'une quelconque des revendications 1 à 3, **caractérisé en ce que** l'anolyte (1) et le catholyte (3) sont mécaniquement séparés par un diaphragme électroconducteur (7).

5. Procédé selon l'une quelconque des revendications 1 à 4, **caractérisé en ce qu'**une solution de séparateur électroconductrice (5) est menée entre deux diaphragmes (7) séparant l'anolyte (1) et le catholyte (3) afin d'empêcher un mélange prématuré de l'anolyte (1) et du catholyte (3).

6. Procédé selon l'une quelconque des revendications 1 à 5, **caractérisé en ce que** le métal de rapport est du cuivre.

7. Procédé selon l'une quelconque des revendications 1 à 5, **caractérisé en ce que** le métal de rapport est sélectionné parmi le groupe suivant : nickel, cobalt, zinc, argent, or, ruthénium, rhodium, palladium, osmium, iridium, platine, manganèse, zirconium, étain, cadmium et indium.

8. Procédé selon l'une quelconque des revendications 1 à 5, **caractérisé en ce que** le métal intermédiaire est du vanadium.

9. Procédé selon l'une quelconque des revendications 1 à 5, **caractérisé en ce que** le métal intermédiaire est sélectionné parmi le groupe titane, chrome et fer.

10. Procédé selon l'une quelconque des revendications 1 à 5, **caractérisé en ce que** le métal intermédiaire est sélectionné parmi le groupe suivant : manganèse, zirconium, molybdène, technétium, tungstène, mercure, germanium, arsenic, sélénium, étain, antimoine, tellure et cuivre.

11. Procédé selon l'une quelconque des revendications 1 à 10, **caractérisé en ce que** la matière d'alimentation contenant le métal de rapport est située dans l'anode (2).

12. Procédé selon l'une quelconque des revendications 1 à 11, **caractérisé en ce que** la solution de départ contient de l'acide sulfurique.

13. Procédé selon la revendication 12, **caractérisé en ce que** la teneur en acide sulfurique dans la solution de départ est d'au moins 50 g/l et de préférence 50 g/l à 1 500 g/l.

14. Procédé selon l'une quelconque des revendications 1 à 13, **caractérisé en ce que** la solution de départ contient de l'acide chlorhydrique ou de l'acide nitrique.

15. Agencement pour produire une poudre de métal de rapport en précipitant la poudre de métal de rapport (14) en mélangeant du métal de rapport dissous avec une solution contenant au moins un métal intermédiaire dans un état d'oxydation inférieur, dans lequel l'agencement comprend une cellule électrolytique contenant du métal de rapport sur un côté anode et du métal intermédiaire dissous sur un côté cathode, pour dissoudre le métal de rapport situé sur le côté anode de la cellule électrolytique et pour l'oxyder dans l'anolyte, et pour réduire le métal intermédiaire dissous situé sur le côté cathode (8) de la cellule électrolytique sur le côté cathode depuis un état d'oxydation supérieur à l'état d'oxydation inférieur ; une chambre de précipitation (12) qui est séparée de la cellule électrolytique ; aussi bien qu'un moyen pour amener une solution d'anolyte et une solution de catholyte respectivement depuis le côté anode (6) de la cellule électrolytique et depuis le côté cathode (8) de la cellule électrolytique jusqu'à la chambre de précipitation (12) pour mélanger le métal de rapport dissous dans l'anolyte et la solution de catholyte contenant le métal intermédiaire réduit, depuis l'extérieur de la cellule électrolytique ; et un moyen pour renvoyer une première partie de la solution en circulation créée suite au mélange de la solution d'anolyte et de la solution de catholyte en retour jusqu'à l'anolyte (1) ; dans lequel la première partie de la solution de départ est composée de la première partie de la solution en circulation ; et un moyen pour renvoyer une seconde partie de la solution en circulation créée suite au mélange de la solution d'anolyte et de la solution de catholyte en retour jusqu'au catholyte (3) ; dans lequel la seconde partie de la solution de départ est composée de la seconde partie de la solution en circulation.

16. Agencement selon la revendication 15, **caractérisé en ce que** la cellule électrolytique comprend un diaphragme électroconducteur (7) entre le côté anode (6) et le côté cathode (8) de la cellule électrolytique pour séparer mécaniquement le côté anode (6) et le côté cathode (8).

17. Agencement selon l'une quelconque des revendications 15 à 16, **caractérisé en ce que** la cellule électrolytique comprend deux diaphragmes électroconducteurs (7) entre le côté anode (6) et le côté cathode (8) de la cellule électrolytique pour séparer mécaniquement le côté anode (6) et le côté cathode (8) au moyen d'une solution de séparateur électroconductrice (5) prévue dans l'espace laissé entre les deux diaphragmes (7).

18. Agencement selon l'une quelconque des revendications 15 à 17, **caractérisé en ce que** le métal de rapport fourni sur le côté anode (6) de la cellule électrolytique est situé dans l'anode (2) de la cellule électrolytique.

19. Agencement selon l'une quelconque des revendications 15 à 18, **caractérisé en ce que** la cellule électrolytique comprend au moins un sac, défini par un diaphragme (7), pour conserver l'anolyte et/ou le catholyte à l'intérieur du sac.

20. Agencement selon la revendication 17, **caractérisé en ce que** la cellule électrolytique comprend un moyen pour mener une solution de séparateur (5) depuis l'espace laissé entre les deux diaphragmes (7) jusqu'au côté anode (6) et/ou jusqu'au côté cathode (8).

21. Agencement selon l'une quelconque des revendications 15 à 20, **caractérisé en ce que** les électrolytes sont placés dans un environnement sans oxygène pour empêcher l'oxydation du métal de rapport et/ou du métal intermédiaire contenu dans les électrolytes.
